

H. A. RICHMOND,  
PROCESS OF TREATING ALUMINOUS ORES.  
APPLICATION FILED NOV. 27, 1916.

1,245,383.

Patented Nov. 6, 1917.



Inventor

Harold A. Richmond

Witnesses

J. V. Skoglund  
A. F. Murray.

By

Howard C. Barlow  
Attorney

# UNITED STATES PATENT OFFICE.

HAROLD A. RICHMOND, OF PROVIDENCE, RHODE ISLAND, ASSIGNOR TO GENERAL ABRASIVE COMPANY, INC., OF NIAGARA FALLS, NEW YORK, A CORPORATION OF NEW YORK.

## PROCESS OF TREATING ALUMINOUS ORES.

1,245,383.

Specification of Letters Patent.

Patented Nov. 6, 1917.

Application filed November 27, 1916. Serial No. 133,551.

To all whom it may concern:

Be it known that I, HAROLD A. RICHMOND, a citizen of the United States, and resident of the city of Providence, in the county of Providence and State of Rhode Island, have invented certain new and useful Improvements in Processes of Treating Aluminous ores, of which the following is a specification.

10 This invention relates to an improved process of treating aluminous ores and more particularly those containing a large percentage of silica.

15 In practice the process heretofore employed for the purpose of treating aluminous ores required the use of an ore such as bauxite which is high in iron and low in silica in order to form magnetic ferrosilicon, whereby these objectionable properties could 20 be readily removed; but the production of such ores, particularly in this country, is limited in quantity, in fact the bauxites found here do not contain sufficient iron in proportion to their silica content to make a 25 magnetic ferrosilicon when fused, without the addition of iron to the charge.

30 The French bauxites are much higher in iron and are, therefore much more readily reduced by the old method, but these bauxites are difficult to obtain and are very expensive.

35 There are, however, among other aluminous ores, large deposits of kaolin found in this country, which may be reduced in a practical way by the employment of my improved process.

40 One object of this invention is to provide a process which is capable of successfully operating upon a greater variety of this 45 character of raw materials to produce the desired quality of abrasives.

45 A further object of the invention is to provide a process whereby the product obtained from such materials possesses greater purity and from which a material of superior commercial quality is produced.

50 A still further object of the invention is, that by my improved process the cost of production is materially lessened as the ore is reduced by the application of heat of a lower temperature and exposed to the heat for a shorter period.

55 With these and other objects in view, the invention consists of certain novel features, as will be more fully described, and particularly pointed out in the appended claims.

In the accompanying drawing.

The figure illustrated in the drawing is a sectional side elevation showing one form of furnace by the use of which my improved process may be successfully carried out.

As is well known aluminous ores occur widely disseminated in nature but in practically all occurrences the ores contain besides the alumina, the oxids of silicon, iron 65 and titanium, either separately or together.

In order to obtain the alumina in a high degree of purity either for the manufacture of aluminum or for abrasive or refractory purposes it is important that these impurities be removed so that a substantially pure alumina results therefrom.

It has been the custom to reduce the impurities to elemental form and thus remove them from the unreduced alumina.

Usually it is sought to make the alloy resulting from the reduction of the impurities high in iron so that it will be magnetic and if the impurities in the aluminous ore are not of such a character as to yield an alloy 80 high in iron sufficient oxid of iron is added to bring this about.

For example there are large deposits of kaolin found in this country which may be successfully used by my improved process 85 as a source of alumina. If these were to be employed as raw material in the familiar process above referred to, the reaction would be as indicated by the following chemical equation:



As will be seen from this equation there is required a very large amount of energy to 95 bring about its reduction and as a consequence it has heretofore been the custom to select ores containing a lower percentage of silica or a higher percentage of iron.

I have discovered that by smelting the 100 aluminous ores with carbonaceous material and sulfur or the sulfid of a base metalliferous element that I can effect the elimination of the silica in a satisfactory and economical manner.

105 I will illustrate my invention with reference to the treating of kaolin and as the basic metalliferous sulfid I will use pyrites or iron sulfid.

110 I take by weight, 182 parts of kaolin, 120 parts of pyrites and 24 parts of carbon. These are intimately mixed together by suit-

able means and then placed in an electric furnace, one form of which is illustrated in the accompanying drawing. The mixture is subjected to electrically developed heat 5 by passing a powerful current through the electrodes 10 and 11, whereby the passage of the current from one to the other forms an arc at 12 which fuses the material, the molten alumina being shown at 13 and the 10 separated and settled molten iron at 14 which may in some cases be drawn off through the tap hole 15. By the application of the heat a reaction takes place which may be expressed by the following equation.



The sulfid of silicon at the reaction temperature is a gas and the silica is thus eliminated. Moreover, since one of the products 20 of the reaction is thus removed from the sphere of action the reaction is driven to the right and there results a perfect elimination of the silicon.

25 The silicon being thus removed as a vapor the metal produced is very high in iron and therefore very magnetic and thus can be effectively removed from the alumina either by being drawn off from the bottom of the furnace or by the use of magnets.

30 If it is desired to use sulfur the reaction takes place according to the following equation:



35 and there results an aluminous product substantially free from impurities.

A study of reaction No. 1 compared with reactions No. 2 and No. 3 shows that there 40 is required a much greater quantity of thermal energy per unit of alumina than in the two latter reactions and moreover we can obtain an elimination of the silica impossible to effect by reaction No. 1.

45 The metal produced as in equation No. 2 is always very high in iron. In consequence it settles out very perfectly from the fused alumina as indicated at 14 in the drawing when it may be readily drawn off 50 and so removed through the tap hole 15.

I do not wish to be restricted to the use of my improved process to the reduction of kaolin as this process may be employed for reducing any aluminous ore to which it may 55 be adapted.

Having thus described one illustrative embodiment of my invention, and the best mode known to me for carrying out my method, I desire it to be understood that although 60 specific terms are employed, they are used in a specific and descriptive sense and not for purposes of limitation, the scope of the invention being defined and limited only by the appended claims.

I claim:

1. The process of forming crystalline alumina, which consists in mixing carbonaceous material and the sulfid of a basic element with aluminous ore, subjecting the mixture to electrically developed heat, and separating the resulting basic element and the crystalline material. 70

2. The process of refining aluminous ores which consists in mixing carbonaceous material and a sulfid with aluminous ore, subjecting the same to electrically developed heat, and removing the impurities as gaseous sulfid. 75

3. The process of refining aluminous ores which consists in mixing carbonaceous material and a sulfid with aluminous ore, subjecting the same to electrically developed heat, and removing the impurities as gaseous sulfid and metal. 80

4. The process of forming crystalline alumina which consists in mixing carbonaceous material and sulfur with aluminous ore, subjecting the mixture to electrically developed heat, and removing the resulting sulfurous compounds and crystalline material separately. 85

5. The process of refining aluminous ores which consists in mixing carbonaceous material and sulfur with the ore, smelting the mixture with electrically developed heat and removing the impurities as gaseous sulfid. 95

6. The process of refining aluminous ores which consists in mixing carbonaceous material and sulfid with the ore, subjecting the mixture to electrically developed heat, and removing the impurities as gaseous sulfid and reduced metal. 100

7. The process of forming crystalline alumina which consists in mixing carbonaceous material and sulfur with aluminous ore, subjecting the mixture to electrically developed heat, and separating the resulting crystalline material and reduced metal. 105

8. The process of refining aluminous ores which consists in mixing carbonaceous material and the sulfid of a basic metal with the ore, subjecting the mixture to electrically developed heat, cooling the resulting product, and separating the crystalline material and reduced metal. 110

9. The process of refining aluminous ores which consists in mixing carbonaceous material and the sulfid of a basic metal with the ore, subjecting the mixture to electrically developed heat, removing the resulting reduced metal in the molten condition, and cooling the product. 115

In testimony whereof I affix my signature in presence of a witness.

HAROLD A. RICHMOND.

Witness:

HOWARD E. BARBER.